# EUROPEAN PATENT SPECIFICATION

(11) **EP 3 486 336 B1**
(45) Date of publication and mention of the grant of the patent: **23.09.2020**
(21) Application number: 17202344.2
(22) Date of filing: 17.11.2017
(51) Int. Cl.: C22B 1/00, C22B 7/00

(54) **METAL-CONTAINING WASTE TREATMENT METHOD**
BEHANDLUNGSVERFAHREN FÜR METALLHALTIGEN ABFALL
PROCÉDÉ DE TRAITEMENT DE DÉCHETS CONTENANT DES MÉTAUX

(43) Date of publication of application: 22.05.2019
(73) Proprietor: Taiheiyo Cement Corporation, Tokyo 135-8578 (JP)
(72) Inventor: TAKEMOTO, Tomonori, Tokyo, 135-8578 (JP); NAKAMURA, Atsushi, Tokyo, 135-8578 (JP); TAKIZAWA, Kou, Tokyo, 135-8578 (JP); ISHIDA, Yasuyuki, Tokyo, 135-8578 (JP)
(74) Representative: Isarpatent

(56) References cited:
- EP-A2- 0 979 677
- DE-A1- 4 205 309
- DE-A1- 19 741 795
- JP-A- H0 947 739
- JP-A- 2000 005 702
- US-A1- 2004 069 687

## Description

### Field of the Invention

The present invention relates to a metal-containing waste treatment method wherein the metal-containing waste also contains waste plastic, and more particularly to a method for properly treating shredder dust such as automobile shredder dust, recovering valuable metal and the like therefrom, and reusing the shredder dust after the valuable metal is recovered as fuel.

### Description of the Related Art

Shredder dust is a mixture of pieces dumped as an industrial waste after waste household electric appliances and waste automobiles are crushed by industrial shredders to recover metals and the like therefrom. Composition of the shredder dust varies in accordance with techniques and facilities of the shredder process and conditions when wastes are previously sorted, so that the composition is not always constant, but main components of the shredder dust consist of resin, foamed urethane, fiber, rubber, and small amount of metal and glass. Shredder dust required to be disposed in controlled landfill sites is requested to be recycled, and mainly in the both fields of thermal and chemical has been developed recycling techniques therefor, and as described in Japanese patent publication No. 2014-205091 gazette for example, in cement industry also, it has been considered to utilize shredder dust as fuel substitute. In addition, in shredder dust are included valuable metals such as iron, nonferrous metals and rare metals, so that it is preferable to easily recover the metals from shredder dust before it is reused.

JP-H09-47739 discloses a metal-containing waste treatment method comprising the steps of
heating a metal-containing waste by burning shredder residue to obtain embrittle waste,
sieving the embrittled waste to obtain an embrittled waste whose particle diameter is less or equal to a predetermined value;
removing a magnetically attractable substance from the embrittled waste whose particle diameter is less or equal to the predetermined value by magnetic sort; and recovering a heavy product from the embrittled waste after the magnetically attractable substance is removed by an air table.

JP-2000-005702 discloses a metal-containing waste treatment method comprising the steps of
heating a metal-containing waste by burning shredder residue to obtain embrittle waste,
removing a magnetically attractable substance from the embrittled waste by magnetic sort;
crushing and sieving the embrittled waste after the magnetically attractable substance is removed to obtain an embrittled waste whose particle diameter is less or equal to a predetermined value; and
recovering a heavy product from the embrittled waste whose particle diameter is less or equal to the predetermined value by jigging machine.

### SUMMARY OF THE INVENTION

### Problems to be Solved by the Invention

However, resin components such as plastic, urethane, rubber, synthetic fiber waste and harness cover in shredder dust are soft (viscoelasticities thereof are high), and the resin components are complexly entangled with metals, so that it is difficult to crush the resin components as they are, to separate and recover the metals therefrom, and to utilize the resin components as fuel substitute.

The present invention has been made in consideration of the above problems, and the object thereof is to recover valuable metal and the like from metal-containing waste such as shredder dust, wherein the metal-containing waste also contains waste plastic, and to reuse it as fuel after the recovery.

### Means of Solving the Problems

In order to attain the object described above, the present invention is a metal-containing waste treatment method characterized by including the steps of: heating a metal-containing waste, which contains waste plastic, at a temperature of 250°C to 400°C to obtain an embrittled waste; crushing or/and sieving the embrittled waste to obtain an embrittled waste whose particle diameter is less or equal to a predetermined value; removing a magnetically attractable substance from the embrittled waste whose particle diameter is less or equal to the predetermined value by magnetic sort; and recovering a heavy product from the embrittled waste after the magnetically attractable substance is removed by an air table.

In addition, the present invention is a metal-containing waste treatment method characterized by including the steps of: heating a metal-containing waste, which contains waste plastic, at a temperature of 250°C to 400°C to obtain an embrittled waste; removing a magnetically attractable substance from the embrittled waste by magnetic sort; crushing or/and sieving the embrittled waste after the magnetically attractable substance is removed to obtain an embrittled waste whose particle diameter is less or equal to a predetermined value; and recovering a heavy product from the embrittled waste whose particle diameter is less or equal to the predetermined value by an air table.

With the both inventions, after heating a metal-containing waste to eliminate entanglement of resins and metals included in the metal-containing waste, sorting is performed, so that recovering noble metals and the like with high quality can be efficiently performed. Further, it is possible to utilize the waste other than the metals as fuel. In addition, when particle diameter of all of the embrittled waste is made less or equal to a predetermined value, the whole embrittled waste can be treated, and recovery efficiencies of the noble metals and the like can be further improved.

In the metal-containing waste treatment method, the embrittled waste immediately before being fed to the air table are sorted into groups with different particle diameters, and from each group is recovered a heavy product by the air table. Subdividing the embrittled waste into groups with different particle diameters to recover a heavy product by the air table enables further improved recovery efficiencies of noble metals and the like.

In addition, when the metal-containing waste is heated a powdery woody body or a granular woody body can be added thereto. Mixing the powdery woody body or a granular woody body into the embrittled waste causes entanglement of resins and metals to be eliminated with ease, which further improves recovery rates of noble metals and so on.

Based on colors of the embrittled waste on the air table can be adjusted operating condition of the air table. With this, based on a point that colors of the embrittled waste such as metals, resins and the like included in the metal-containing waste are different from each other and a point that in the metals exist a metal whose color is different from those of others, the waste can be sorted by colors, which can improve sorting accuracy and can efficiently treat the metal-containing waste.

Based on colors of the embrittled waste on the air table can be adjusted position of a partition board attached to a discharging port of the air table.

The embrittled waste immediately before being fed to the air table can be sorted by wind force to remove a light material, and the embrittled waste after the light material is removed can be fed to the air table. With this, it is possible to recover magnetically attractable substances such as iron and mainly light materials other than metals from the waste before feeding to the air table, which can further improves sorting accuracy of the metal-containing waste.

In addition, together with the metal-containing waste may be fed another metal-containing waste whose metal content is higher than the metal-containing waste to the air table. With this, even when metal content of the metal-containing waste is low, it is possible to visually recognize, with ease, a boundary line between metals and wastes other than metals in color distribution of the metal-containing waste on the air table, resulting in further improved sorting accuracy.

The metal-containing waste or/and the other metal-containing waste may include resin, which enables preferable treatment of automobile shredder dust or the like.

From the light material obtained by the wind force sort and from a light product obtained by the air table can be recovered resins embrittled by the heating as fuels.

### Effects of the Invention

As described above, with the present invention, valuable metal can be recovered from metal-containing waste such as shredder dust, and the waste can be reused as fuel.

### BRIEF DESCRIPTION OF THE DRAWINGS

Figure 1 is a flowchart for explaining the metal-containing waste treatment method according to the first embodiment of the present invention;
Figure 2 shows an example of an air table used for the metal-containing waste treatment method according to the present invention, wherein (a) is an schematic perspective view showing a condition before a metal-containing waste is treated, and (b) is an schematic top view showing a condition when the metal-containing waste is actually treated;
Figure 3 is a flowchart for explaining the metal-containing waste treatment method according to the second embodiment of the present invention;
Figure 4 is a flowchart for explaining the metal-containing waste treatment method according to the third embodiment of the present invention;
Figure 5 is a flowchart for explaining the metal-containing waste treatment method according to the forth embodiment of the present invention; and
Figure 6 is a flowchart for explaining the metal-containing waste treatment method according to the fifth embodiment of the present invention.

### DESCRIPTION OF THE EMBODIMENTS

Next, embodiments for carrying out the present invention will be explained with reference to the drawings. In the following explanation, a case that shredder dust as a metal-containing waste is treated will be explained as an example.

The shredder dust (hereinafter abbreviated as "dust") is, for example, a waste that is discharged under a condition that waste plastic and other wastes are mixed, and as the shredder dust, automobile shredder dust, constructive plastic waste and the like are typical examples. Here, the waste plastic is a waste of synthetic highpolymer body, and includes wastes of synthetic resin molded body, seat-shaped material, tape-shaped material, strap-shaped material, sponge-shaped material and particulate, synthetic fiber and synthetic rubber. In addition, the other wastes include waste of metal and/or soil and stone (such as glass, concrete, tile, ridge tile, pottery, inorganic building material and sediment) at least, and in addition to those, can include wastes of paper, natural fiber, wood, tatami mat, leather, oil and fat, sludge, incineration ash, carbon, ceramic, liquid material, sludge material and the like.

Figure 1 shows a treatment device 1 for carrying out the metal-containing waste treatment method according to the first embodiment of the present invention, and the treatment device 1 is provided with: a heater 2 for heating a received dust D1; a crusher 3 for crushing a heated dust D2; a sieving machine 4 for sieving a crushed dust D3; a magnetic force sorting device (hereinafter abbreviated as "magnetic sorter") 5 for removing a magnetically attractable substance from a sieved fine particle (under sieve) D4; a wind force sorting device (hereinafter abbreviated as "wind sorter") 6 for removing a light material from a dust D6 after the magnetically attractable substance is removed; a magnetic sorter 7 for removing a magnetically attractable substance from dust D7 after the light material is removed; and an air table 8 for performing dry type gravity sorting for a dust D8 after the magnetically attractable substance is removed.

The heater 2 is installed to heat the received dust D1 at 250°C to 400°C to embrittle resin (waste other than metal) in the dust D1, and as the heater 2 can be used a fixed furnace, a stoker furnace, a rotary kiln furnace, a fluidized bed furnace, a vertical furnace, a multistage furnace or the like. The heating treatment may be performed in air atmosphere, oxidizing atmosphere, reducing atmosphere or inert atmosphere, but performing it in oxidizing atmosphere is preferable because mechanical strength of the dust D1 can be decreased in a shorter time in comparison to other atmospheres.

With the heating of the dust D1 by the heater 2, fixed carbon content of the resin in the dust D1 becomes high, and brown and black particles increase. On the other hand, much metal waste in the dust D1 generates oxide film thereon to become light brown or brown, and embrittled resin fusing to the metal waste coats the metal waste to make it brown or black, so that metallic luster on the metal waste disappears.

The crusher 3 is installed to crush the heated dust D2, and as the crusher 3 can be used a hummer crusher, an impact crusher, a jaw crusher, a roll crusher, a cutter mill, a roller mill, an autogenous grinder or the like. In view of wear property and sizing property against metal mixed in the dust D2, impact-type hummer crushers or impact crushers are preferably used.

As the sieving machine 4 can be used a vibration sieve, a rotary screen or the like, and the sieving machine 4 is not particularly restricted as far as it has openings of X mm and can separate the crushed dust D3 into the coarse particle (on sieve) D5 whose size is more or equal to Xmm and the fine particle (under sieve) D4 whose size is less than Xmm.

As the magnetic sorters 5, 7 can be used a hanging-type or a drum-type sorter with a permanent magnet.

The wind sorter 6 is a device for sorting by difference in terminal speeds between the sorted objects, and kinds thereof are not particularly limited, and as the wind sorter 6, as far as it can sort the dust D6 into a light material and a heavy material can be used a vertical type, an internal circulation type, a zig zag type and so on.

It is particularly preferable that the wind sorter 6 has a construction for arbitrarily changing a sorting point of the light material and the heavy material. Since components of the dust D6 vary to a certain extent, it is preferable to operate the wind sorter 6 while the sorting point described above is properly adjusted in order to preferably balance between that the light material after the wind sorting is easily converted to fuel by the crushing and that the light material converted to fuel is secured as much as possible.

The air table 8 is installed to apply dry type gravity sorting to the dust D8. The air table 8 is mounted, as shown in Fig. 2(a), to sort the dust D8 into a light product L1, a heavy product H1, and a middle weight product M1 having a specific gravity between these products by the dry type gravity sorting, and is provided with: a vibratory table 8a, inclining at predetermined inclination angles θ1 (end slope) and θ2 (side slope), with small vent holes for air A for vibrating in directions of bidirectional arrows V; a blowing up type blower (not shown) for supplying the air A through rotation from the lower surface of the vibratory table 8a to the upper surface thereof; partition boards 8c, 8d as boundaries of each product discharged from an end portion 8b of the vibratory table 8a; and so on. In addition, to the air table 8 is mounted a dust collector (not shown) such as a cyclone, and the lightest matter in the dust D8 is blown up by airflow to be recovered as a cyclone dust CD.

Meanwhile, when the dust D8 after the magnetically attractable substance is removed is fed to the air table 8, it is preferable to subdivide the dust D8 into groups with different particle sizes, and to separately feed these particle groups to the air table 8. With this, recovery accuracies of noble metals and copper can be improved. For example, when size of the dust D8 is less than 8mm the dust D8 is fed to sieving devices with 5mm and 2mm openings in this order, which sorts the dust D8 into a particle group whose particle diameter is less than 8mm and more or equal to 5mm, a particle group whose particle diameter is less than 5mm and more or equal to 2mm, and a particle group whose particle diameter is less than 2mm. Then, the particle group whose particle diameter is less than 8mm and more or equal to 5mm, the particle group whose particle diameter is less than 5mm and more or equal to 2mm, and the particle group whose particle diameter is less than 2mm are separately fed to the air table 8, and the dust D8 may be separately treated in accordance with the particle diameter ranges. In this connection, classification diameter of the particle diameter ranges can be properly adjusted as far as the classification diameter is less or equal to X mm.

Next, the metal-containing waste treatment method of the present embodiment will be explained with reference to Figs. 1 and 2.

Firstly, a received dust D1 is fed to the heater 2 to be heated, and an embrittled dust D2 is obtained. Applying heating treatment at the above temperature to the dust D1 allows mechanical strength thereof to be decreased to embrittle it, but it is preferable to make relationship between the heating temperature and the heating time inverse proportion such that when the heating temperature is set to be 300°C, the heating time is set to be 1.5 hours; when the temperature is set to be 350°C, the time is set to be 1 hour; and when the temperature is set to be 400°C, the time is set to be 45 minutes. In addition, since desirable relationship between the heating temperature and the heating time varies with size of the dust D1, kinds of resin therein, and other conditions, it is preferable to properly adjust the relationship.

In the heating treatment of the dust D1, it is preferable to mix a powdery woody body, a granular woody body or a crushed woody body into the dust D1 because entanglement of resin and metal can be eliminated and recovery ratio of metal improves. As the powdery woody body, the granular woody body woody or the crushed woody body are listed plant fibers such as wood waste, bamboo waste and coconut husk, and it is preferable to use the wood waste in the plant fibers because the wood waste can be easily ground when being recovered together with the light product. It is preferable that mixing ratio of the powdery woody body, the granular woody body woody or the crushed woody body is 10 to 30 mass percent of the whole matter including the dust D1.

Next, the embrittled dust D2 is fed to the crusher 3 to be crushed, and a dust D3 discharged from the crusher 3 is fed to the sieving machine 4 to be sorted into a fine particle D4 and a coarse particle D5. Then, returning the coarse particle D5 to the crusher 3 to grind it again can obtain the fine particle D4 whose size is less than Xmm. Meanwhile, when large mass, that is, particle whose size is 20mm for example generates in the dust D2, it is preferable to previously crush and disintegrate it. In addition, without returning the coarse particle D5 to the crusher 3, only the fine particle D4 sieved in the sieving machine 4 may be fed to the magnetic sorter 5.

It is preferable to set Xmm of openings of the sieving machine 4 such that, in order to secure preferable sorting accuracy in the following air table 8, a dust whose particle diameter is 0.5 to 10 mm in the crushed dust D3 becomes more than 60 weight percent of the whole crushed dust D3, and when the whole crushed dust D3 is treated at one time it is preferable to set X 6 to 9. Because there is a possibility that sorting accuracy in the air table 8 decreases when a particle whose particle diameter is less than 0.5 mm is too much, or when a particle whose particle diameter is more or equal to 10 mm is too much.

From the whole dust D2 or the sieved coarse particle D5 whose size is more or equal to X mm are previously removed metals as much as possible, which can improve crushing efficiency of the crusher 3. The metal sorting can be performed by magnetic sorting, eddy current sorting, sorter sorting or the like.

The eddy current sorting is a method of sorting nonferrous metal such as aluminum from the dust D2 and the like by utilizing a difference in repulsive forces based on eddy currents. For example, in an eddy current sorting device, through interaction between induced current and moving magnetic field that generate inside due to electromagnetic induction action caused by moving magnetic field of a rotating magnetic body mounted on a front end side of a conveyer belt, a thrust is added to a shredder dust transported on the front end side of the conveyer belt in a rotating direction of the rotating magnetic body, and nonferrous metal or the like is made bounce out from the surface of the conveyer belt in a direction of the resultant force of this thrust and the gravity acted to the nonferrous metal or the like. As the eddy current sorting device is preferably used a magnet rotation type, a direct belt conveyor type or a cylinder rotation type device.

The fine particle D4 is fed to the magnetic sorter 5, and a magnetic metal such as iron is magnetically collected in the magnetic sorter 5 to be removed. The fine particle D4 includes metal waste, and final target is to recover noble metals such as gold and silver therefrom, so that general-purpose metal such as iron that is magnetically attractable substance is sorted and removed from the fine particle D4.

Next, the dust D6 from the magnetic sorter 5 is fed to the wind sorter 6 to remove a light material. Previously removing light material can reduce load in shape sorting in the air table 8 in a post stage, resulting in improved recovery accuracy of noble metals. When the dust D6 is sorted by wind force, as light materials are mainly separated soft waste plastic, fiber and the like, and as heavy materials are mainly separated metal waste, soil and stone waste, large-diameter hard waste plastic and the like. Then, the dust D7 after the light materials are removed is fed to the magnetic sorter 7, and in the magnetic sorter 7 is removed the magnetically attractable substance such as iron, and the dust D8 from the magnetic sorter 7 is fed to the air table 8.

As shown in Fig. 2(a), the dust D8 is fed onto the vibratory table 8a of the air table 8, and by the vibration of the vibratory table 8a and the air A supplied from a blowing-up type blower, on the vibratory table 8a, as shown in Fig. 2(b) are formed flows of the light product L1, the middle weight product M1 and the heavy product H1, and by the partition boards 8c, 8d, these products L1, M1, H1 are separately discharged from the end 8b of the vibratory table 8a.

Here, the partition boards 8c, 8d are mounted at the positions of the boundary lines among the products L1, M1, H1 that are predicted based on property of the dust D8, so that when the property of the dust D8 is deferent from that being predicted, the positions of boundary lines among the products L1, M1, H1 in the end portion 8b of the air table 8 are deferent from those being predicted. As a result, there is a possibility that into a material discharged from the air table 8 as the light product L1 may be mixed the middle weight product M1 and the heavy product H1.

Then, in the present embodiment is visually confirmed color distributions of the dust D8, and based on the color distributions are adjusted positions of the partition boards 8c, 8d. Here, the color distributions generate due to substantially three colors of brown or block based on fixed carbon of the light product L1, silver based on aluminum of the middle weight product M1 and copper based on copper of the heavy product H1. In addition, in such a manner that the boundary lines of the color distributions become clear and flows of the light product L1, the middle weight product M1 and the heavy product H1 have constant widths are adjusted θ1, θ2, amount of the air A and frequency of the vibratory table 8a.

Here, the light product L1 obtained in the air table 8 is an embrittled material of resin and the like, and the middle weight product M1 is aluminum and glass, and the heavy product H1 is copper and noble metals such as gold and silver. In addition, the lightest material is blown up by air flow to be recovered by a cyclone. Further, as the heavy product H1 are recovered lead and chromium that are cement repellents, which decreases amount of the cement repellents mixed into cement as the following fuel.

Meanwhile, when in the air table 8 may be mixed a small amount of copper and the like into the middle weight product M1 and a small amount of aluminum may be mixed into the heavy product H1, in such cases, the middle weight product M1 and the heavy product H1 are separately treated in a gravity sorter or a color sorter, and the copper and the like are removed from the middle weight product M1, and from the heavy product H1 is removed aluminum.

In addition, when metal content of the received dust D1 is low, there is a possibility that materials on the air table 8 uniformly become brown or block and colors of the metals on the air table 8 cannot be visually confirmed. In such a case, a waste including a certain amount of metal is fed onto the air table 8, which can make visual confirmation of colors of the metals that have been originally included in the dust D1 easier.

Further, applying eddy current sorting to the heavy product H1 obtained by the air table 8 can make noble metal concentration high. When a magnet rotation type eddy current sorting device is used, it is preferable to make rotational speed of a drum more than 4000rpm. With this, it is possible to efficiently recover noble metals as conductors from the heavy product H1 whose size is small.

In addition, a material other than the heavy product H1 by the air table 8 is recovered as fuel. In other words, the light material recovered by the wind sorter 6 and the cyclone dust CD, the light product L1 and the middle weight product M1 recovered by the air table 8 contribute reuse as fuel, so that the dust and others are recovered as fuel. When utilized as fuel, they are ground in advance to be less or equal to 3 mm, more preferably less or equal to 1mm, further preferably less or equal to 0.1 mm.

Further, from the fine particle D4 discharged from the sieving machine 4 and the dust D8 after the magnetically attractable substance is removed in the magnetic sorter 7 also, in order to improve recovery efficiency of noble metals, it is preferable to recover nonferrous metal such as aluminum by the eddy current sorting.

As described above, with the present embodiment, from shredder dust are recovered noble metals such as gold, silver and copper. In addition, recovered materials other than the heavy product H1 recovered by the air table 8 are recovered as fuel. The fuel obtained as described above is preferably used after chlorine is removed therefrom, that is, desalting is performed. The desalting is performed by water washing or the like.

In addition, in the present embodiment are focused on a point that the metals included in the received dust D1 and the embrittled material of resin and the like are different in color with each other and a point that in metals exist metals whose colors are different from each other, and based on the colors can be adjusted operating condition of the air table 8, so that it is possible to handle a case that the property of the waste changes, and sorting accuracy of the shredder dust can be improved.

Next, the second embodiment of the present invention will be explained with reference to Fig. 3.

A treatment device 10 according to the present embodiment is provided with, in addition to the heater 2 to the air table 8 in the first embodiment shown in Fig. 1, a magnetic sorter 11 for removing a magnetically attractable substance from a coarse particle (on sieve) D5 of the sieving machine 4; a sieving machine 12 for sieving a dust D9 after the magnetically attractable substance is removed; an eddy current sorter 13 for collecting a nonferrous metal from a fine particle (under sieve) D10 discharged from the sieving machine 12; an electromagnetic induction sorter 15 for recovering a stainless steel from a dust D11 discharged from the eddy current sorter 13; and an eddy current sorter 14 for recovering a nonferrous metal from a coarse particle (on sieve) D12 discharged from the sieving machine 12.

As the magnetic sorter 11, like the magnetic sorters 5, 7 in the first embodiment can be used a hanging type or drum type sorter with a permanent magnet or the like. In addition, as the sieving machine 12, like the sieving machine 4 in the first embodiment can be used a vibration sieve, a rotary screen or the like.

The eddy current sorters 13, 14 are, as described above, devices for sorting nonferrous metal such as aluminum by utilizing a difference in repulsive forces based on eddy currents, and as the eddy current sorters 13, 14 can be used magnet rotation type, direct belt conveyor type or cylinder rotation type devices. Meanwhile, when the magnet rotation type eddy current sorter is used rotational speed of a drum may be less or equal to 4000 rpm.

When an object body passes a magnetic field, an eddy current generates due to electromagnetic induction, and a current value depends on the conductivity of the object body. The electromagnetic induction sorter 15 utilizes this phenomenon, and detects the eddy current by using a magnetic field sensor and sorts object bodies by identifying kinds of the object bodies through computer analysis based on the difference in the current value.

Meanwhile, after the eddy current sorting, metals can be collected by a vertical mill while grinding the metals. The vertical mill is a device for grinding, drying and separating into a fine powder and a course powder against a raw waste, and finally sorts into a mill product on fine particle side with a predetermined particle diameter distribution and a mill discharge on course powder side with a larger predetermined particle diameter distribution (refer to Japanese patent application 2016-89196 gazette).

Next, a metal-containing waste treatment method in the present embodiment will be explained with reference to Fig. 3.

In the first embodiment is returned the coarse particle D5 from the sieving machine 4 to the crusher 3, but in the present embodiment is fed the coarse particle D5 to the magnetic sorter 11, and in the magnetic sorter 11 is magnetically collected and removed a magnetic metal such as iron.

Next, the dust D9 discharged from the magnetic sorter 11 is fed to the sieving machine 12 so as to be sieved into a fine particle D10 whose size is less than 30mm and a coarse particle D12 whose size is more or equal to 30mm, and the fine particle D10 and the coarse particle D12 are separately fed to the eddy current sorters 13, 14 to recover nonferrous metals such as aluminum and copper therefrom. Further, dusts D11, D13 from the eddy current sorters 13, 14 are fed to the electromagnetic induction sorter 15 to recover stainless steels. At last, a dust D14 is manually sorted to obtain a nonferrous metal and a residue. The residue is for being utilized as fuel. In addition, amount of recovered nonferrous metal is not much, but the nonferrous metal is that recovered from the products after the magnetic sorting and the like as previous processes, so that the nonferrous metal has a sufficient concentration as recycled raw material, which improves recovery rate of the nonferrous metal as the whole.

In the present embodiment, in the sieving machine 4 is sieved the dust D3 into a dust whose size is more or equal to Xmm and a dust whose size is less than Xmm (X=2 to 10), and after the sieving the dust D3 is sieved into the fine particle D4 whose size is less than Xmm under the sieve and the coarse particle D5 whose size is more or equal to Xmm on sieve, but when the X is 5 to 10, in order to improve sorting accuracy after the magnetic sorter 5, it is preferable to sieve the fine particle D4 into a dust whose size is more or equal to Ymm and a dust whose size is less than Ymm, and the dusts are preferably fed to the following devices 5 to 8.

Next, the third embodiment of the present invention will be explained with reference to Fig. 4.

In a treatment device 20 according to the present embodiment, in the heater 2 to the magnetic sorter 7 in the first embodiment shown in Fig. 1, the sieving machine 4 is arranged in a later stage of the magnetic sorter 7 as a sieving machine 21, and the treatment device 20 is provided with air tables 22, 23 for separately performing dry type gravity sorting to a fine particle (under sieve) D27 and a coarse particle (on sieve) D28 from the sieving machine 21 in a later stage of the sieving machine 21.

As the air tables 22, 23 can be used the same ones as the air table 8 shown in Fig. 2, and the air table 22 separates the fine particle D27 into a light product L21, a heavy product H21, and a middle weight product M21 having a specific gravity between these products, and the air table 23 separates the coarse particle D28 into a light product L22 and a heavy product H22.

Next, a treatment method of shredder dust in the present embodiment will be explained with reference to Fig. 4. Meanwhile, a dust D21 that is treated in the present embodiment includes 1% or more aluminum and 1% or more copper to the whole dust D21, and openings of the sieving machine 21 are set to be 5 mm (X=5).

Motions of the heater 2, the crusher 3, the magnetic sorter 5, the wind sorter 6 and the magnetic sorter 7 are the same as those in the first embodiment, and the received dust D21 is heated in the heater 2, and a heated dust D22 is crushed in the crusher 3, and from a crushed dust D23 is removed a magnetically attractable substance by the magnetic sorter 5, and from a dust D24 after the magnetically attractable substance is removed is removed a light material by the wind sorter 6, and from a dust D25 after the light material is removed is removed a magnetically attractable substance by the magnetic sorter 7.

Next, a dust D26 from the magnetic sorter 7 is fed to the sieving machine 21 so as to be sieved into a fine particle D27 and a coarse particle D28, and the fine particle D27 is fed to the air table 22 to be sieved into a light product L21, a middle weight product M21 and a heavy product H21, and the coarse particle D28 is fed to the air table 23 to recover a light product L22 and a heavy product H22.

Sieving motion in the air table 22 is the same as that in the air table 8 in the first embodiment. On the other hand, when the coarse particle D28 is sorted into the light product L22 and the heavy product H22 by dry type gravity sorting in the air table 23 also, based on color distributions of the coarse particle D28 is adjusted a partition board (not shown) of the air table 23.

Here, the light products L21, L22 obtained by the air tables 22, 23 are embrittled materials such as resin and the like, and the middle weight product M21 obtained by the air table 22 is aluminum and glass, and the heavy product H21 obtained by the air table 22 is copper and noble metals such as gold and silver, and the heavy product H22 obtained by the air table 23 is aluminum.

In addition, in the same manner as the air table 8 in the first embodiment, there is a possibility that in the air table 22 are mixed a small amount of copper and the like into the middle weight product M21 and a small amount of aluminum is mixed into the heavy product H21. In such cases, the middle weight product M21 and the heavy product H21 are separately treated in a gravity sorter or a color sorter, and from the middle weight product M21 are removed copper and the like, and from the heavy product H21 is removed aluminum.

In addition, when metal content of the received dust D21 is low, there is a possibility that the materials on the air tables 22, 23 uniformly become brown or block and colors of the metals on the air tables 22, 23 cannot be visually confirmed. In such a case, wastes including a certain amount of metal are fed onto the air tables 22, 23, which can make visual confirmation of colors of the metals that have been originally included in the dust D2 easier.

Further, in the present embodiment, two partition boards 8c, 8d are mounted on boundary lines among products L21, M21 and H21. But, the present invention is not limited to the case, and only one partition board 8c may be mounted on the boundary line between the middle weight product M21 and the light product L21. In this case, sorting is performed under a condition that the middle weight product M21 and the heavy product H21 coexist, so that an aluminum in the middle weight product M21 and a copper in the heavy product H21 are sorted by a gravity sorter or a color sorter.

In addition, the dust D21 described above includes 1% or more aluminum and 1% or more copper to the whole dust D21. But, when an aluminum in the dust D21 is 1% or more and a copper therein is less than 1% to the whole dust D21, the dust D21 includes much metals other than copper such as iron, nickel and noble metal as the heavy product H21.

Here, since most of the metals other than copper does not have metallic luster, it is impossible to use the metals as a guide to determine a place where the partition board 8d is mounted, but aluminum has metallic luster, so that based on the metallic luster of aluminum can be mounted the partition boards 8c, 8d on the boundary lines of the products L21, M21 and H21. In this case, the partition board 8c may be mounted between the heavy product H21 and the middle weight product M21, and the partition board 8d may be mounted between the middle weight product M21 and the light product L21, or one partition board 8c may be mounted on the boundary line between the middle weight product M21 and the light product L21. When one partition board is mounted, sorting is performed under a condition the middle weight product M21 and the heavy product H21 coexist, so that an aluminum in the middle weight product M21 and metals in the heavy product H21 are sorted by a gravity sorter or a color sorter.

In addition, when aluminum in the dust D21 is less than 1% and copper therein is 1% or more to the whole dust D21, it is impossible to use the metallic luster of the aluminum as a guide to determine places where the partition boards 8c, 8d are mounted, but base on the metallic luster of copper can be distinguished the light product L21 and the heavy product H21, so that between the light product L21 and the heavy product H21 can be mounted one partition board 8c. In the sorted heavy product H21 is mixed an embrittled material of small amount of resin and the like, so that the heavy product H21 is treated by a gravity sorter or a color sorter, and from the heavy product H21 is removed an embrittled material of resin and the like.

Meanwhile, in this case, in the light product L21 is mixed a small amount of copper and the like, and in order to recover the copper and the like, it is necessary to feed total amount of the light product L21 to a gravity sorter or a color sorter, but it is difficult to perform the treatment because amount of the light product L21 is large.

Then, it is preferable to add the dust D21 or a waste with high aluminum content to the dust D27 before it is fed to the air table 22 such that aluminum content of the dust D27 becomes 1% or more to treat the dust D27. With this, between the light product L21 and the heavy product H21 is formed an area of the middle weight product M21, which can prevent copper and the like from mixing into the light product L21.

In addition, when aluminum and copper in the dust D21 are less than 1% to the whole weight of the dust D21, only the light product L21 can be confirmed, and preferable positions for recovering the middle weight product M21 and the heavy product H21 are not judged, so that it becomes difficult to determine mounting positions of the partition boards 8c, 8d.

In this case, a waste including aluminum or/and copper is added to the dust D21 or the dust D27 before it is fed to the air table 22, and contents of aluminum and copper are made to 1% or more, which allows areas of the middle weight product M21 and the heavy product H21 to generate clearly, so that preferable positions where the partition boards 8c, 8d are mounted can be determined.

Meanwhile, wastes including much aluminum are cloth wastes with ornaments such as fasteners and buttons, aluminum electrolytic capacitors electrically mounted on substrates, and so on. In addition, wastes including much copper (including brass and nickel silver) are cloth wastes with ornaments such as fasteners and buttons, and electrical wire connectors, USB cables, modular plugs, coated copper wires, and so on.

In addition, operation of the air table 22 is fed back so as to increase the heavy product H21 such as copper and noble metals in accordance with a condition that the heavy product H21 is recovered. In concrete, positions of the partition boards 8c, 8d of the air table 22, frequency of the vibratory table 8a, inclination angles θ1, θ2 of the vibratory table 8a, amount of air of the vibratory table 8a and others are fed back in accordance with a condition that the heavy product H21 is recovered. Meanwhile, recovery condition of the heavy product H21 is judged by measuring bulk specific gravity of the recovered heavy product H21 for example.

Next, the forth embodiment of the present invention will be explained with reference to Fig. 5.

The treatment device 30 according to the present embodiment is different from the treatment device 20 according to the third embodiment in that by the sieving machine 31 is divided a dust D36 into three particles consisting of a fine particle D39, a middle size particle D40 and a coarse particle D41, and the fine particle D39, the middle size particle D40 and the coarse particle D41 are treated by air tables 32, 33 and 34 respectively. Explanations of the same construction as the treatment device 20 other than the above are omitted. As the sieving machine 31 can be used a vibration sieve, a rotary screen or the like, and each air table 32, 33, 34 has the same construction as the air table 8.

The fine particle D39 is less than 2mm in diameter, the middle size particle D40 more or equal to 2mm and less than 5mm in diameter, and the coarse particle D41 is more than 5mm in diameter.

The fine particle D39 is divided into a light product L33 and a heavy product H33 by the air table 32. The light product L33 is glass, and the heavy product H33 is copper and noble metals. A partition board is mounted between flows of the light product L33 and the heavy product H33 based on color of copper to enable the sorting.

The middle size particle D40 is divided into a light product L34, a middle weight product M34 and a heavy product H34 by the air table 33. The light product L34 is an embrittled material such as resin, and the middle weight product M34 is aluminum and glass, and the heavy product H33 is copper and noble metals. A partition board is mounted between flows of the light product L34 and the middle weight product M34 based on color of aluminum to enable the sorting, and a partition board is mounted between flows of the middle product M34 and the heavy weight product H34 based on color of copper to enable the sorting.

The coarse particle D41 is divided into a light product L35 and a heavy product H35 by the air table 34. The light product L35 is an embrittled material such as resin, and the heavy product H35 is aluminum. A partition board is mounted between flows of the light product L35 and the heavy product H35 based on color of aluminum to enable the sorting.

In the present embodiment also are focused on a point that colors of the embrittled wastes such as metals, resins and the like included in a shredder dust of waste automobile are different from each other and a point that in metals exist metals whose colors are different from each other, and based on the colors can be adjusted operating conditions of the air tables 32, 33 and 34, so that it is possible to handle a case that the property of the waste changes, and sorting accuracy of the shredder dust can be improved.

Next, the fifth embodiment according to the present invention will be explained with reference to Fig. 6.

The treatment device 50 according to the present embodiment is different from the treatment device 20 according to the third embodiment in that the dust D56 after the magnetically attractable substance is removed by the magnetic sorter 7 is sorted in two stages by air tables 51, 52 without sieving sort. Each air table 51, 52 has the same construction as the air table 8. Explanations of the same construction as the treatment device 20 other than the above are omitted.

The dust D56 after the magnetically attractable substance is removed by the magnetic sorter 7 is fed to the air table 51 to be sorted into a light product L56 and a heavy product H56. The light product L56 is an embrittled material such as resin, and a heavy product H56 is a mixture of aluminum, glass, copper and noble metals. A partition board is mounted between flows of the light product L56 and the heavy product H56 based on colors of aluminum and copper to enable the sorting.

Then, the heavy product H56 is fed to the air table 52 to be sorted into a light product L57, a middle weight product M57 and a heavy product H57. The light product L57 is glass, and the middle weight product M57 is aluminum, and the heavy product H57 is copper and noble metals. A partition board is mounted between flows of the light product L57 and the middle weight product M57 based on color of aluminum to enable the sorting, and a partition board is mounted between flows of the middle product M57 and the heavy weight product H57 based on color of copper to enable the sorting.

In the present embodiment also are focused on a point that colors of the embrittled wastes such as metals, resins and the like included in a shredder dust of waste automobile are different from each other and a point that in metals exist metals whose colors are different from each other, and based on the colors can be adjusted operating conditions of the air tables 51, 52, so that it is possible to handle a case that the property of the waste changes, and sorting accuracy of the shredder dust can be improved.

Meanwhile, in the embodiment described above is explained a case that a shredder dust is treated as an example, but the present invention can treat various metal-containing wastes other than shredder dust.

### [Examples]

Hereinafter, examples of the present invention will be explained in detail.

(Example 1) First, 2514 kg of automobile shredder dust was prepared, and to the automobile shredder dust was added a slaked lime. Next, to an antler kiln heated to 320°C was fed the automobile shredder dust with a feeding speed of 30 kg/h to perform heating treatment. After the treatment, 1961kg of embrittled shredder dust was obtained.

1889 kg of the embrittled shredder dust obtained as described above was fed to a magnetic sorter (hanging type) and a sieving machine (vibration sieve) with 5mm openings to be sieved into that whose size was 5mm or more (on sieve) and that whose size was less than 5mm (under sieve).

Next, from the embrittled shredder dust whose size was less than 5mm were removed a magnetically attractable substance and a light material by a magnetic sorter (hanging type) and a wind sorter (internal circulation type). Next, by an air table (manufactured by TRIPLE/S DYNAMICS, INC.) was recovered a heavy product that can be sufficiently used for raw materials of noble metals (gold, silver) and copper. Particularly, recovery ratio of gold reached 75%. The recovered metals and masses thereof are shown in the following Table 1.

**[Table 1]**

| | | CONCENTRATION (GOLD·SILVER:g/t, COPPER·ALUMINUM:%) | | | | RECOVERY RATIO (%) FROM SHREDDER DUST | | | |
|---|---|---|---|---|---|---|---|---|---|
| | RECOVERY AMOUNT (kg) | GOLD | SILVER | COPPER | ALUMINUM | GOLD | SILVER | COPPER | ALUMINUM |
| HEAVY PRODUCT | 6.43 | 131 | 540 | 56 | 2 | 75 | 9 | 5 | 0.1 |
| NONFERROUS METAL | 43 | 0.4 | 190 | 9 | 48 | 2 | 21 | 6 | 8 |
| MANUALLY SORTED NONFERROUS METAL | 1. 35 | <0.1 | 16 | 44 | 6 | - | 0. 1 | 1 | 0. 1 |

On the other hand, from the embrittled shredder dust, whose size was 5mm or more, on sieve were removed metals other than iron (manually sorted nonferrous metal) by manual sorting at first. Next, magnetic sorting and sieve sorting (30mm) were performed, and both of materials on sieve and under sieve were fed to an eddy current sorting device (magnet rotation type, rotational speed 3000 rpm) to remove nonferrous metal such as aluminum and copper therefrom. Further, manual sorting or the like was applied to obtain a residue. The residue is used as fuel. Although recovered amount of the obtained nonferrous metal was not much, the nonferrous metal was recovered from products after the manual sorting and the magnetic sorting were performed in previous processes, so that the nonferrous metal had sufficient concentration of metals as a recycling material, and recovery ratio of the nonferrous metal on the whole could be improved. Further, concentration and recovery ratio of silver were relatively high.

To the light material, the light product and the cyclone dust after the wind force sorting, in order to evaluate combustibleness (weight reduction ratio after combustion for a predetermined period of time) against pulverized coal as a main fuel for a cement kiln, combustion tests were performed with a tubular electric furnace (42mm in diameter, 1450°C in temperature, atmosphere air flow rate: 1L/min, amount of sample: 1g). The weight reduction ratios after the combustion tests are shown in Table 2. A pulverized coal continuously decreased in weight reduction ratio for 0.5 to 4 minutes. On the other hand, every embrittled material did not change in weight reduction ratio for 0.5 to four minutes, which could judge that combustibles of the materials were almost completely burnt for 0.5 minutes. As a result, it is confirmed that each embrittled material is better than pulverized coal in combustibility, and the embrittled material can be used in place of pulverized coal as fuel without problems. In addition, amounts recovered by sorting are shown in the following Table 2.

**[Table 2]**

| | RECOVERY AMOUNT (kg) | BURNING TIME (minute) | | | |
|---|---|---|---|---|---|
| | | 0.5 | 1 | 2 | 4 |
| RESIDUE OBTAINED BY SORT | 604 | 64 | 67 | 68 | 68 |
| LIGHT MATERIAL | 811 | 50 | 54 | 57 | 56 |
| LIGHT PRODUCT | 90 | 40 | 38 | 40 | 43 |
| CYCLONE DUST | 7 | 55 | 55 | 55 | 57 |
| PULVERIZED COAL | | 29 | 38 | 59 | 75 |
| (%) | | | | | |

(Example 2) At first, 650kg of an automobile shredder dust was prepared, and to the automobile shredder dust was added wood chips and a slaked lime. The ratio of the automobile shredder dust and the wood chips is 70 to 30. In heating treatment of the shredder dust, a powdery woody body or a granular woody body was preferably mixed to the shredder dust since entanglement of resins and metals was eliminated to improve recovery ratio of metals. As the powdery woody body or the granular woody body are listed vegetable fibers such as wood chips, bamboo waste and coconut shell, among them, wood chips are preferably used since when recovered together with a light product they can be ground with ease.

Next, to the antler kiln with 325°C of inner temperature was thrown an automobile shredder dust at a rate of 30kg/h to be heated for embrittling treatment. After the treatment, 520kg of embrittled shredder dust was obtained.

510kg of embrittled shredder dust that was obtained by the above treatment was fed to a hammer-type crusher with a screen with 8mm openings for crushing. After the crushing, 510kg of embrittled shredder dust whose largest particle diameter was 8mm or less was obtained. As for this embrittled shredder dust, ratio of particles whose particle diameter were between 0.5-5mm to the whole particles exceeded 60 weight %.

Meanwhile, when the embrittled shredder dust was fed to a hammer-type crusher with a screen with 5mm openings for crushing, particles whose particle diameter was 0.5mm or less were much, and noble metals would also be ground finely, which was judged not to be preferable. Particle diameter distributions before and after the grinding are shown in the following Table 3.

**[Table 3]**

| EMBRITTLED MATERIAL | GRAIN SIZE DISTRIBUTION (%) | | | | | | | |
|---|---|---|---|---|---|---|---|---|
| | <0.5mm | 0.5-1mm | 1-2mm | 2-5mm | 5-10mm | 10-20mm | 20-40mm | 40mm< |
| BEFORE CRUSHING | 11 | 8 | 6 | 15 | 12 | 16 | 29 | 3 |
| AFTER CRUSHING 5mm | 51 | 26 | 17 | 6 | 0 | 0 | 0 | 0 |
| AFTER CRUSHING 8mm | 34 | 21 | 23 | 19 | 3 | 0 | 0 | 0 |

505kg of an embrittled shredder dust after the grinding were sorted with a magnetic sorter (hanging type) and a wind sorter (internal circulation type) to remove a magnetically attractable substance (No.1 magnetically attractable substance), which could be used as a ferrous raw material, and a light material (dust sorted by wind force sorting), which could be used as a fuel. Next, using a magnetic sorter (hanging type), a magnetically attractable substance (No.2 magnetically attractable substance), which could be used as a ferrous raw material, was removed.

Next, with an air table (made by TRIPLES/S DYNAMICS, INC. (USA), a heavy product mainly containing noble metals (gold and silver) and copper, a middle weight product mainly containing aluminum and a light product mainly containing an emblittled material such as resin that could be used for fuel, were recovered. In addition, a dust contained in an air generating by the air table and mainly containing an embrittled material such as resin was recovered by a cyclone (cyclone dust). In order to clarify boundary lines among the heavy product, the middle weight product and the light product based on colors of aluminum and copper on the air table, θ1 (end slope) was adjusted between 2-15°, θ2 (side slope); 0-6°, air feed rate; 0.5-3m/s, and table frequency; 4-10Hz in accordance with operating conditions.

At an end of the air table, a boundary line between the heavy product and the middle weight product, and a boundary line between the middle weight product and the light product were visually confirmed, and partition boards were mounted at the boundary lines. With this, at an end portion with 1800mm of total width, widths of flows of the heavy product, the middle weight product and the light product became 75mm, 225mm and 1500mm respectively.

Bulk specific gravities and metal contents of the automobile shredder dust, the embrittled material, the product obtained by crushing the embrittled material and the embrittled material fed to the air table are shown in Table 4.

**[Table 4]**

| | BULK SPECIFIC GRAVITY (-) | Au (g/t) | Ag (g/t) | Cu (%) | Al (%) |
|---|---|---|---|---|---|
| AUTOMOBILE SHREDDER DUST | 0.23 | 0.3 | 21 | 1. 3 | 1. 2 |
| EMBRITTLED MATERIAL | 0.35 | 0.3 | 26 | 1. 7 | 1.5 |
| PRODUCT OBTAINED BY CRUSHING EMBRITTLED MATERIAL | 0.62 | | | | |
| EMBRITTLED MATERIAL FED TO AIR TABLE | - | 0.4 | 31 | 2.5 | 1. 7 |

Products recovered through sorting process from 505kg of embrittled shredder dust after the crushing are shown in Table 5.

**[Table 5]**

| | RECOVERY AMOUNT (kg) | RECOVERY RATIO (%) |
|---|---|---|
| No.1 MAGNETICALLY ATTRACTABLE SUBSTANCE | 20 | 4 |
| WIND SEPARATED DUST | 150 | 32 |
| No. 2 MAGNETICALLY ATTRACTABLE SUBSTANCE | 2 | <1 |
| LIGHT PRODUCT | 231 | 49 |
| MIDDLE WEIGHT PRODUCT | 19 | 4 |
| HEAVY PRODUCT | 13.8 | 3 |
| CYCLONE DUST | 39 | 8 |

Bulk specific gravity, total calorific value and metal contents of each product are shown in Table 6.

**[Table 6]**

| | BULK SPECIFIC GRAVITY | TOTAL CALORIFIC VALUE | Au | Ag | Cu | Al |
|---|---|---|---|---|---|---|
| | (-) | (kcal/kg) | (g/t) | (g/t) | (%) | (%) |
| No. 1 MAGNETICALLY ATTRACTABLE SUBSTANCE | 1. 85 | - | 1.6 | 29 | 0.8 | 0.3 |
| WIND SEPARATED DUST | 0. 50 | 3, 990 | <0.1 | 16 | 0. 2 | 1.1 |
| No. 2 MAGNETICALLYATTRACTABLE SUBSTANCE | 1. 29 | - | 2. 6 | 38 | 1.1 | 0.7 |
| LIGHT PRODUCT | 0.57 | 4, 110 | <0.1 | 12 | 0. 3 | 1.1 |
| MIDDLE WEIGHT PRODUCT | 0.81 | 2, 770 | 1.1 | 15 | 3.8 | 5.6 |
| HEAVY PRODUCT | 1. 56 | - | 6. 6 | 417 | 42. 6 | 8.7 |
| CYCLONE DUST | 0.58 | 3, 840 | <0.1 | 11 | 0.5 | 1. 2 |

Metal distribution rates of each product are shown in Table 7.

**[Table 7]**

| | Au (%) | Ag (%) | Cu (%) | Al (%) |
|---|---|---|---|---|
| No.1 MAGNETICALLY ATTRACTABLE SUBSTANCE | 21 | 5 | 2 | 1 |
| WIND SEPARATED DUST | 0 | 20 | 3 | 24 |
| No. 2 MAGNETICALLY ATTRACTABLE SUBSTANCE | 3 | 1 | 0 | 0 |
| LIGHT PRODUCT | 0 | 23 | 10 | 36 |
| MIDDLE WEIGHT PRODUCT | 14 | 2 | 9 | 15 |
| HEAVY PRODUCT | 61 | 47 | 74 | 17 |
| CYCLONE DUST | 0 | 3 | 2 | 7 |

Results shown in Tables 6 and 7 mean that gold, silver and copper are much in the heavy product and the heavy product is proved to be useful as refining raw material. In the middle weight product are included copper and aluminum, but concentrations thereof are low, so that it can be refining raw materials by further processes for separately sorting copper and aluminum. Colorific values of the dust sorted by wind force (light material), the light product and the cyclone dust are high, so that they can be used as fuels together with the residue after a copper and an aluminum are sorted from the middle weight product.

### Description of the Reference Numerals

1, 10, 20, 30, 50 treatment devices
2 heater
3 crusher
4, 12, 21, 31 sieving machines
5, 7, 11 magnetic sorters
6 wind sorter
8, 22, 23, 32, 33, 34, 51, 52 air tables
13, 14 eddy current sorters
15 electromagnetic induction sorter

## Claims

1. A metal-containing waste treatment method comprising the steps of:
heating a metal-containing waste, which contains waste plastic, at a temperature of 250°C to 400°C, to obtain an embrittled waste;
crushing or/and sieving the embrittled waste to obtain an embrittled waste whose particle diameter is less or equal to a predetermined value;
removing a magnetically attractable substance from the embrittled waste whose particle diameter is less or equal to the predetermined value by magnetic sort; and
recovering a heavy product from the embrittled waste after the magnetically attractable substance is removed by an air table.

2. A metal-containing waste treatment method comprising the steps of:
heating a metal-containing waste, which contains waste plastic, at a temperature of 250°C to 400°C to obtain an embrittled waste;
removing a magnetically attractable substance from the embrittled waste by magnetic sort;
crushing or/and sieving the embrittled waste after the magnetically attractable substance is removed to obtain an embrittled waste whose particle diameter is less or equal to a predetermined value; and
recovering a heavy product from the embrittled waste whose particle diameter is less or equal to the predetermined value by an air table.

3. The metal-containing waste treatment method as claimed in claim 1 or 2, wherein the embrittled waste immediately before being fed to the air table are sorted into groups with different particle diameters, and from each group is recovered a heavy product by the air table.

4. The metal-containing waste treatment method as claimed in claim 1, 2 or 3, wherein when the metal-containing waste is heated a powdery woody body or a granular woody body is added thereto.

5. The metal-containing waste treatment method as claimed in one of claims 1 to 4, wherein based on colors of the embrittled waste on the air table is adjusted operating condition of the air table.

6. The metal-containing waste treatment method as claimed in claim 5, wherein based on colors of the embrittled waste on the air table is adjusted position of a partition board attached to a discharging port of the air table.

7. The metal-containing waste treatment method as claimed in one of claims 1 to 6, wherein the embrittled waste immediately before being fed to the air table is sorted by wind force to remove a light material, and the embrittled waste after the light material is removed is fed to the air table.

8. The metal-containing waste treatment method as claimed in one of claims 1 to 7, wherein together with the metal-containing waste is fed another metal-containing waste whose metal content is higher than the metal-containing waste to the air table.

9. The metal-containing waste treatment method as claimed in one of claims 1 to 8, wherein the metal-containing waste or/and the other metal-containing waste include resin.

10. The metal-containing waste treatment method as claimed in claim 9, wherein from the light material obtained by the wind force sort and from a light product obtained by the air table are recovered resins embrittled by the heating as fuels.

## Patentansprüche

1. Verfahren zur Behandlung von metallhaltigem Abfall, umfassend die folgenden Schritte:
Erhitzen eines metallhaltigen Abfalls, der Kunststoffabfall enthält, auf eine Temperatur von 250°C bis 400°C, um einen versprödeten Abfall zu erhalten;
Zerkleinern oder/und Sieben des versprödeten Abfalls, um einen versprödeten Abfall zu erhalten, dessen Teilchendurchmesser kleiner oder gleich einem vorbestimmten Wert ist;
Entfernen einer magnetisch anziehbaren Substanz aus dem versprödeten Abfall, dessen Teilchendurchmesser kleiner oder gleich einem vorbestimmten Wert ist, durch magnetische Sortierung; und
Rückgewinnung eines schweren Produkts aus dem versprödeten Abfall, nachdem die magnetisch anziehbare Substanz durch einen Lufttisch entfernt wurde, durch einen Lufttisch.

2. Verfahren zur Behandlung von metallhaltigem Abfall, umfassend die folgenden Schritte:
Erhitzen eines metallhaltigen Abfalls, der Kunststoffabfall enthält, auf eine Temperatur von 250°C bis 400°C, um einen versprödeten Abfall zu erhalten;
Entfernen einer magnetisch anziehbaren Substanz aus dem versprödeten Abfall durch magnetische Sortierung;
Zerkleinern oder/und Sieben des versprödeten Abfalls, nachdem die magnetisch anziehbare Substanz entfernt wurde, um einen versprödeten Abfall zu erhalten, dessen Partikeldurchmesser kleiner oder gleich einem vorbestimmten Wert ist; und
Rückgewinnung eines schweren Produkts aus dem versprödeten Abfall, dessen Partikeldurchmesser kleiner oder gleich dem vorgegebenen Wert ist, durch einen Lufttisch.

3. Verfahren zur Behandlung von metallhaltigem Abfall nach Anspruch 1 oder 2, wobei der versprödete Abfall unmittelbar vor der Zuführung zum Lufttisch in Gruppen mit unterschiedlichen Partikeldurchmessern sortiert wird und aus jeder Gruppe ein schweres Produkt durch den Lufttisch zurückgewonnen wird.

4. Verfahren zur Behandlung von metallhaltigem Abfall nach Anspruch 1, 2 oder 3, wobei beim Erhitzen des metallhaltigen Abfalls ein pulverförmiger, holziger Körper oder ein granulatförmiger, holziger Körper hinzugefügt wird.

5. Verfahren zur Behandlung von metallhaltigem Abfall nach einem der Ansprüche 1 bis 4, wobei auf der Grundlage der Farben des versprödeten Abfalls auf dem Lufttisch der Betriebszustand des Lufttisches eingestellt wird.

6. Verfahren zur Behandlung von metallhaltigem Abfall nach Anspruch 5, bei dem auf der Grundlage der Farben des versprödeten Abfalls auf dem Lufttisch die Position einer Trennwand eingestellt wird, die an einer Auslassöffnung des Lufttisches angebracht ist.

7. Verfahren zur Behandlung von metallhaltigem Abfall nach einem der Ansprüche 1 bis 6, bei dem der versprödete Abfall unmittelbar vor seiner Zuführung zum Lufttisch durch Windstärke sortiert wird, um ein leichtes Material zu entfernen, und der versprödete Abfall nach der Entfernung des leichten Materials dem Lufttisch zugeführt wird.

8. Verfahren zur Behandlung von metallhaltigem Abfall nach einem der Ansprüche 1 bis 7, wobei zusammen mit dem metallhaltigen Abfall ein anderer metallhaltiger Abfall, dessen Metallgehalt höher ist als der metallhaltige Abfall, dem Lufttisch zugeführt wird.

9. Verfahren zur Behandlung von metallhaltigem Abfall nach einem der Ansprüche 1 bis 8, wobei der metallhaltige Abfall oder/und der andere metallhaltige Abfall Harz enthält.

10. Verfahren zur Behandlung von metallhaltigem Abfall nach Anspruch 9, bei dem aus dem leichten Material, das durch die Windkraftsortierung erhalten wird, und aus einem leichten Produkt, das durch den Lufttisch erhalten wird, Harze, die durch das Erhitzen versprödet sind, als Brennstoffe zurückgewonnen werden.

## Revendications

1. Procédé de traitement de déchet contenant du métal comprenant les étapes consistant à :
chauffer un déchet contenant du métal, qui contient du plastique de déchet, à une température de 250 °C à 400 °C,
pour obtenir un déchet fragilisé ;
broyer et/ou tamiser le déchet fragilisé pour obtenir un déchet fragilisé dont le diamètre de particule est inférieur ou égal à une valeur prédéterminée ;
enlever une substance magnétiquement attractive du déchet fragilisé dont le diamètre de particule est inférieur ou égal à la valeur prédéterminée par tri magnétique ; et
récupérer un produit lourd du déchet fragilisé après que la substance magnétiquement attractive ait été enlevée par une table à air.

2. Procédé de traitement de déchet contenant du métal comprenant les étapes consistant à :
chauffer un déchet contenant du métal, qui contient du plastique de déchet, à une température de 250 °C à 400 °C pour obtenir un déchet fragilisé ;
enlever une substance magnétiquement attractive du déchet fragilisé par tri magnétique ;
broyer et/ou tamiser le déchet fragilisé après que la substance magnétiquement attractive ait été enlevée pour obtenir un déchet fragilisé dont le diamètre de particule est inférieur ou égal à une valeur prédéterminée ; et
récupérer un produit lourd du déchet fragilisé dont le diamètre de particule est inférieur ou égal à une valeur prédéterminée par une table à air.

3. Procédé de traitement de déchet contenant du métal selon la revendication 1 ou 2, dans lequel le déchet fragilisé immédiatement avant d'être alimenté à la table à air est trié en groupes avec des tailles de particules différentes, et à partir de chaque groupe est récupéré un produit lourd par la table à air.

4. Procédé de traitement de déchet contenant du métal selon la revendication 1, 2 ou 3, dans lequel, lorsque le déchet contenant du métal est chauffé, un corps boisé poudreux ou un corps boisé granulaire y est ajouté.

5. Procédé de traitement de déchet contenant du métal selon l'une des revendications 1 à 4, dans lequel la condition de fonctionnement de la table à air est ajustée sur la base des couleurs du déchet fragilisé sur la table à air.

6. Procédé de traitement de déchet contenant du métal selon la revendication 5, dans lequel la position d'un circuit de séparation attaché à une porte de déchargement de la table à air est ajustée sur la base des couleurs du déchet fragilisé sur la table à air.

7. Procédé de traitement de déchet contenant du métal selon l'une des revendications 1 à 6, dans lequel le déchet fragilisé immédiatement avant d'être alimenté à la table à air est trié par la force du vent pour enlever un matériau léger, et le déchet fragilisé après que le matériau léger ait été enlevé est alimenté à la table à air.

8. Procédé de traitement de déchet contenant du métal selon l'une des revendications 1 à 7, dans lequel conjointement avec le déchet contenant du métal est alimenté un autre déchet contenant du métal dont la teneur en métal est supérieure au déchet contenant du métal à la table à air.

9. Procédé de traitement de déchet contenant du métal selon l'une des revendications 1 à 8, dans lequel le déchet contenant du métal ou/et l'autre déchet contenant du métal comportent de la résine.

10. Procédé de traitement de déchet contenant du métal selon la revendication 9, dans lequel à partir du matériau léger obtenu par le tri par la force du vent et à partir d'un produit léger obtenu par la table à air sont récupérées les résines fragilisées par le chauffage comme combustibles.
